

## UNITED STATES PATENT OFFICE

2,347,543

## ALLOY FOR PERMANENT MAGNETS

Walter Dannöhl and Hans Neumann, Berlin-Siemensstadt, Germany; vested in the Alien Property Custodian

No Drawing. Application October 27, 1937, Serial No. 171,214. In Germany January 7, 1937

5 Claims. (Cl. 175—21)

Our invention relates to an alloy for permanent magnets.

It is known to employ as material for the manufacture of permanent magnets alloys of cobalt, nickel and copper and alloys of iron, nickel and copper. The just-mentioned magnets of cobalt, nickel and copper are described in our U. S. Patent No. 2,170,047, granted August 22, 1939, on our copending application Serial No. 111,252, filed November 17, 1936, of which this is a continuation-in-part. These magnets have excellent magnetic qualities such as a potential coercive force above 100 oersted together with the advantage of being machineable by cutting tools and having a higher mechanical strength than other high grade magnets.

According to the present invention, similar advantages are obtained by employing alloys of cobalt, nickel, copper and iron for producing permanent magnets. Magnets of this composition have considerably better magnetic properties than the known iron-nickel-copper alloys, and are advantageous even in comparison with ternary nickel-cobalt-copper alloys, since by virtue of the iron content they may have a cheaper composition and also present improved working properties.

Magnets according to our present invention contain 1 to 35% iron, 10 to 45% nickel, 1 to 70% cobalt, and 20 to 80% copper.

Alloys containing 5 to 25% iron, 15 to 35% nickel, 5 to 40% cobalt and 30 to 60% copper show especially favorable magnetic properties. The magnetic properties of magnets according to the invention are further enhanced if the alloys are first heated above 1000° C., then quenched and finally reheated to a temperature between 500 and 750° C.

The improvement of the magnetic properties attained by alloys according to the invention will become apparent from the following table referring to a number of examples of different composition.

| Alloy No. | Fe | Ni | Co | Cu | B <sub>r</sub> | H <sub>e</sub> | B <sub>r</sub> .J.H <sub>e</sub> .10 <sup>-5</sup> |
|-----------|----|----|----|----|----------------|----------------|----------------------------------------------------|
| 1a        | 35 | 25 | —  | 40 | 4,600          | 80             | 3.7                                                |
| 1b        | 10 | 25 | 25 | 40 | 4,800          | 280            | 13.5                                               |
| 2a        | 30 | 30 | —  | 40 | 4,300          | 140            | 6.0                                                |
| 2b        | 15 | 30 | 15 | 40 | 5,000          | 220            | 11.0                                               |
| 2c        | 5  | 30 | 25 | 40 | 4,300          | 405            | 17.4                                               |
| 3a        | 40 | 20 | —  | 40 | 5,100          | 30             | 1.5                                                |
| 3b        | 10 | 20 | 30 | 40 | 5,600          | 240            | 13.5                                               |
| 4a        | 16 | 28 | —  | 56 | 3,200          | 280            | 9.0                                                |
| 4b        | 9  | 28 | 7  | 56 | 2,900          | 395            | 11.5                                               |
| 5a        | 27 | 28 | —  | 45 | 4,300          | 150            | 6.4                                                |
| 5b        | 20 | 28 | 7  | 45 | 4,300          | 240            | 10.3                                               |
| 6a        | 20 | 23 | —  | 57 | 3,640          | 367            | 13.3                                               |
| 6b        | 13 | 23 | 7  | 57 | 3,250          | 463            | 15.1                                               |

In the first column of this table are indicated

60

the alloys of which those designated by *a* refer to iron-nickel-copper, whereas the alloys *b* and *c* are obtained from the alloys *a* by substituting cobalt for a portion of iron. The last three columns of the table indicate the values of the remanence, the coercive force and the magnetic power B<sub>r</sub>.J.H<sub>e</sub>.10<sup>-5</sup>. Particularly noteworthy is the great increase of the coercive force present in every case. Thus, for instance, with an alloy containing 40% iron, 20% nickel and 40% copper, the coercive force increases from 30 to 240 oersted if cobalt is substituted for 30% iron. At the same time also the remanence increases by 10% from 5,100 to 5,600 gauss. The improvement is also apparent from the increase in the magnetic power B<sub>r</sub>.J.H<sub>e</sub> from 1.5.10<sup>5</sup> to 12.6.10<sup>5</sup>.

In some cases, such as in examples 1b and 2b, the substitution of cobalt for iron effects not only an increase in the coercive force, but also an increase in the remanence. In other cases, such as in alloy 5b, the remanence is not affected, and in some cases a decrease of the remanence is noticeable, as will be seen from alloys 4b and 6b showing a decrease of approximately 10%. In the last-mentioned case, the coercive force is considerably increased so that the product of these two magnitudes shows a considerable improvement of the magnetic properties as compared to the known iron-nickel-copper alloys.

The alloys designated by *a* were produced with the most favorable heat treatment in order to attain the best possible magnetic properties. The alloys designated by *b* and *c* were produced in such a manner that the material was at first heated for 10 hours at a temperature of 1,050° and 1,100° centigrade respectively, then quenched in oil, annealed for 1 to 40 hours at a temperature of 600° to 700° centigrade and finally cooled down to room temperature. The fluctuations in the annealing period are found necessary, since different compositions required different periods for obtaining the best magnetical properties. For other compositions than given in the table, departures from these periods and temperatures may appear appropriate.

The alloys may contain small amounts of reducing materials, for instance, about 1% manganese, small quantities of silicon, magnesium, aluminum or beryllium, or several of such common additions.

What is claimed is:

1. A permanent magnet formed of an alloy containing 5 to 25% iron, 15 to 35% nickel, 5 to 40% cobalt, and a balance consisting substantially of 30 to 60% copper, besides minor amounts of customary additions and impurities, and being magnetized up to a coercive force above 100 oersted and a remanence above 1,000 gauss.
2. A permanent magnet formed of an alloy

comprising 30 to 60% copper, the remainder consisting of substantially all iron, nickel and cobalt in minimum amounts of 5% iron, 15% nickel and 5% cobalt.

3. A permanent magnet formed of an alloy comprising 1 to 30% iron, 10 to 45% nickel, 5 to 70% cobalt, and a balance of 20 to 80% consisting substantially of copper.

4. A permanent magnet consisting substantially of 1 to 30% iron, 10 to 45% nickel, 5 to 70% cobalt and 20 to 80% copper besides small amounts of customary additions and impurities,

and being magnetized to a magnetic power above  $10^6$ .

5. A permanent magnet formed of an alloy containing 1 to 30% iron, 10 to 45% nickel, 5 to 70% cobalt and a balance of 20 to 80% consisting substantially of copper, and exhibiting a magnetic power above  $10^6$  upon quenching from above 1000° C. and tempering between 500 and 750° C.

10

WALTER DANNÖHL.  
HANS NEUMANN.